

Oct. 25, 1949.

M. H. BARNES ET AL

2,485,553

FILAMENT GUIDE

Filed May 23, 1944



INVENTORS  
MALCOLM H. BARNES  
EDWARD L. McCANDLESS  
BY *Schaeferwald*  
ATTORNEY

## UNITED STATES PATENT OFFICE

2,485,553

## FILAMENT GUIDE

Malcolm H. Barnes and Edward L. McCandless,  
Kenmore, N. Y., assignors to The Linde Air  
Products Company, a corporation of Ohio

Application May 23, 1944, Serial No. 536,964

11 Claims. (Cl. 242—157)

1

The principal object of this invention is the provision of novel filament guides having improved resistance to the wearing and cutting action of rapidly moving filaments such as thread, yarn, wire, and ribbon. Another object is the provision of a novel filament guide having such a long life that a relatively high initial cost will be more than offset by the relatively low cost per yard of filament passing over the guide, hereinafter called the unit cost.

Large textile mills require thousands of thread guides to guide and support the thread during its passage from one operation to another. Thread guides constructed in accordance with the prior art wear out quite rapidly and require frequent replacement, especially when the thread is impregnated with an abrasive material, such as titania, as is often done with rayon and other synthetic fibers. Among the many materials which have been used for thread guides in the prior art are cobalt-chromium-tungsten alloy, borosilicate glass, porcelain, soft glass, stainless steel, nickel-chromium wire, and sintered alumina, but none of these materials has given completely satisfactory results. The principal objections to these materials are their relatively low resistance to the wearing and cutting action of rapidly moving thread, and their relatively high unit cost. Furthermore, a worn or cut thread guide, which is often detected too late, may damage many yards of thread before replacement is made. Similar undesirable conditions have long existed in industries manufacturing and using metal wire.

The present invention will be readily understood from the following detailed description having reference to the accompanying drawing, wherein:

Figs. 1 and 2 are enlarged side and end elevational views, respectively, of a pigtail type of filament guide;

Figs. 3 and 4 are elevational views of two other types of filament guides, Fig. 4 being greatly enlarged.

Figs. 5 and 6 are enlarged side elevational views of two other types of filament guides, used as thread tensioning devices; and

Fig. 7 is a greatly magnified longitudinal sectional view of a fragment of one type of filament guide.

In the following description the term "filament guide" is used to denote any type of device for guiding and supporting filaments such as textile threads, metal wire, and yarns, as well as ribbon-like filaments, regardless of whether the device is used solely as a guide or has secondary functions, such as stretching or tensioning the

2

filament. Furthermore, although several specific types of filament guides are described in detail, this is by way of illustration only. The principles of the invention are applicable to filament guides in general, regardless of shape or construction. A few examples of filament guides are simple guides, tensioning posts, the orifice guides of steam stretching chambers, and the eyes of needles and shuttles.

10 We have found that a filament guide having at least a filament contacting portion comprising a unicrystalline body of material selected from the group consisting of corundum and spinel, either natural or synthetic, is far superior to the filament guides of the prior art in its resistance to wearing and cutting, as well as in its low unit cost. Corundum, of course, is substantially pure alumina, best known as natural or synthetic crystalline rubies and sapphires; and 15 the spinel used is a magnesia-alumina crystal which may contain between 8% and 28% of magnesia, the balance being substantially all alumina. Synthetic corundum and spinel single crystals are made either as large boules or as 20 thin long rods by the method, or variations thereof, fundamentally disclosed in Verneuil Patent 1,004,505, by dropping alumina or alumina-magnesia powder through a gas flame, and accumulating and solidifying the fused material on a 25 suitable support.

The filament guides of the invention are particularly advantageous when they have glossy, scratch-free filament contacting surfaces substantially identical with the surface produced by 30 intensely heating a rough surface layer of a spinel or corundum body until the desired finish is obtained. It is thought that the rough surface portions fuse and coalesce in the heat to form the desired glossy, continuous, smooth, and 35 scratch-free surface. However, it is possible that the surface is heat glossed by a solid diffusion mechanism. Heating may be accomplished by a gas flame, in a furnace, or in any other desired manner.

40 Another method for heat glossing a spinel or corundum filament guide is to apply to a rough surface a thin film of an addition agent, such as an oxide or oxide-forming compound, fulfilling at least one of the following requirements: 45 having a lower melting point than the guide material, forming a eutectic with the guide material, forming a solid solution with the guide material, and forming a low melting peritectic with the guide material. The film is then bonded 50 to the original surface by heating the body intensely in any suitable way. Here also it is not known for certain whether the glossing action 55

proceeds by melting the material, or by a solid diffusion mechanism. Addition agents suitable for glossing corundum and spinel filament guides in this way include calcium oxide, magnesia, sodium oxide, and silica.

Heat glossed surfaces resist wear and cutting by filaments such as thread, yarn, and wire much better than do unglossed surfaces or abrasively polished surfaces. The small crevices in unglossed surfaces and the minute scratches always existing on abrasively polished surfaces act as concentration points for the wearing and cutting action of the filament as it passes over the thread guide.

It is especially desirable to form our novel filament guides from long, thin, homogeneous rods of material selected from the group consisting of corundum and spinel, because of the adaptability of such rods for this type of device. Such rods, usually having a diameter of three sixteenths inch or smaller as grown by a variation of the fundamental Verneuil process, can be used in the straight condition in the manner shown in Fig. 6 of the drawing. They are most advantageous for filament guides, however, when they are formed into shapes especially designed for guiding filaments. For example, a rod of corundum or spinel can be bent to form a filament guiding bight or loop simply by heating a portion of the rod in a flame to its softening point, and then applying force transversely of the longitudinal axis of the rod. It is advantageous, to reduce friction and wear, that such guides be polished either with abrasives or by heat glossing, preferably the latter which increases resistance of the guides to wearing and cutting by the filament. Heat glossing generally occurs spontaneously over that portion of the rod which is heated for forming it into a special shape.

Figs. 1 and 2 show details of a mounted pigtail type filament guide comprising a horizontally mounted homogeneous rod 11 of corundum or spinel bent through 360° into the form of a bight 12, and mounted in a supporting sleeve 13 in position for the passage of a filament 15 through the bight.

Fig. 3 shows a different form of filament guide 17 consisting of a homogeneous corundum or spinel rod bent through 180° to form a J-shaped bight 18, which may be mounted in any suitable manner to guide a filament through the bight. It is evident that rods having bights of different shapes than those shown in Figs. 1 to 3, such as closed bights and eyes, are useful as filament guides.

Fig. 4 shows a disc shaped filament guide 19 of corundum or spinel having a V-notch 21. Such a guide is usually shaped from a large piece of corundum or spinel by cutting and grinding, after

which the roughly ground surfaces forming the notch 21 are heat glossed for greater resistance to wearing and cutting by the filament.

The guide shown in Fig. 5 is a tensioning device comprising a rod 35 of corundum or spinel having a neck portion 37 of reduced cross-sectional area, which has been formed by heating the central portion of the rod to plasticity and then stretching the rod. Due to the heat, the neck 37 has a heat glossed surface free from scratches. The rod 35 is mounted adjacent to its ends in two sleeves 39 and 41, and the filament 42 is wound one or more times around the neck 37 to maintain a desired tension on the filament during its passage, while preventing the filament from wandering along the length of the guide.

In Fig. 6 the guide or tensioning device for guiding a filament 49 is a straight homogeneous rod 43 of corundum or spinel mounted similarly to the rod of Fig. 5 in sleeves 45 and 47 adjacent to the ends of the device. It is desirable to have a heat glossed scratch-free surface on the rod 43, but the unpolished rod in the condition "as grown" also has far superior resistance to wear than the materials used for filament guides in the prior art. Moreover, the straight rod shown in Fig. 6 can be provided with either a smooth fully glossed surface, or with a partially glossed wavy scratch-free surface having smooth undulations, as shown on a greatly magnified scale at 51 on the fragment of a rod 53 in Fig. 7. Such a wavy surface can be produced by heating the surface of the "as grown" rod until the many small crystal projections on the rod are rounded off, and then discontinuing heating before the attainment of an even, completely glossed surface. Another procedure for forming a wavy surface is to overheat the rod. A wavy surface is of particular value for straight guides and tensioning devices, and in the trade the wavy surface is sometimes spoken of as giving less friction.

The following table shows the results of accelerating abrasion tests carried out on spinel and corundum rod filament guides, in comparison with rod filament guides of other materials. In these tests 150 denier synthetic vinyl resin yarn was passed through a 4% suspension of titania and through a tensioning device before being drawn over the guide under test. The yarn made a right angle turn on the guide and a tension of 30 to 35 grams was maintained on the yarn as it traveled over the guide at 167 yards per minute. A total of 80,160 yards of yarn was drawn across each guide. The figures in the table are approximate but sufficiently accurate to provide a fair comparison among the several thread guides.

|      | Guide Material                | Approx. Diam. of Guide, inches (D) | Finish                      | First Evidence of Cutting, Yards (Y) | Y/D     |
|------|-------------------------------|------------------------------------|-----------------------------|--------------------------------------|---------|
| (1)  | Synthetic sapphire            | 0.10                               | Heat glossed                | 23,380                               | 234,000 |
| (2)  | do                            | 0.14                               | do                          | 25,050                               | 179,000 |
| (3)  | do                            | 0.23                               | do                          | 35,070                               | 152,000 |
| (4)  | do                            | 0.28                               | Diamond polished (400 mesh) | 25,050                               | 90,000  |
| (5)  | do                            | 0.15                               | Heat glossed                | 16,700                               | 111,000 |
| (6)  | do                            | 0.29                               | Diamond polished (600 mesh) | 25,050                               | 87,000  |
| (7)  | Sintered Alumina              | 0.25                               |                             | 15,050                               | 60,000  |
| (8)  | do                            | 0.24                               |                             | 10,020                               | 42,000  |
| (9)  | Co-Cr-W alloy                 | 0.18                               |                             | 7,515                                | 39,000  |
| (10) | Borsilicate glass             | 0.186                              |                             | 4,175                                | 22,000  |
| (11) | Soft glass                    | 0.125                              |                             | 2,505                                | 20,000  |
| (12) | Porcelain                     | 0.42                               |                             | 5,010                                | 12,000  |
| (13) | Stainless Steel (18 Cr, 8 Ni) | 0.093                              |                             | 1,670                                | 18,000  |
| (14) | Nickel-Chromium wire          | 0.09                               |                             | 2,450                                | 27,000  |

It is apparent that the spinel and the sapphire (corundum) filament guides were far superior to the other guides tested, especially when the factor of size variation is eliminated. This superiority is emphasized and rationalized as in the column headed Y/D, by dividing by the guide diameter the number of yards of thread passed over the guide before the first evidence of cutting was observed.

Several types of filament guides have been described specifically above to illustrate the principles of the invention. It is to be understood that the invention is not limited to such specific types but that changes in construction and arrangement can be made within the scope of the appended claims.

We claim:

1. A filament guide comprising a unicrystalline body of material selected from the group consisting of corundum and spinel, said body having a glossy scratch-free filament contacting surface substantially identical with the surface produced by intensely heating such a body.

2. A filament guide according to claim 1, wherein said body is corundum.

3. A filament guide according to claim 1, wherein said body is magnesia-alumina spinel.

4. A filament guide according to claim 1, wherein said body is a long thin rod.

5. A filament guide comprising a unicrystalline rod of material selected from the group consisting of corundum and spinel, said rod having a bight for the passage of a filament, said bight having a glossy scratch-free filament-contacting surface substantially identical with the surface produced by intensely heating a surface layer of such rod.

6. A filament guide comprising a straight unicrystalline rod composed of material selected from the group consisting of corundum and spinel, said rod having a glossy scratch-free filament-contacting surface substantially identical with the surface produced by intensely heating a surface layer of such a rod.

7. A filament guide comprising a unicrystalline rod composed of material selected from the group consisting of corundum and spinel, said rod having a filament-contacting neck section of gradually reduced cross-sectional area, said neck section having a glossy, scratch-free surface substan-

tially identical with the surface produced by intensely heating a surface layer of such a rod.

8. A filament guide having at least a filament-contacting portion comprising a unicrystalline body of material selected from the group consisting of corundum and spinel, said body having a glossy scratch-free surface produced by heat bonding to the original body at least one oxide fulfilling at least one of the following requirements: having a melting point lower than such material, forming a eutectic with such material, forming a solid solution with such material, and forming a low melting peritectic with such material.

9. A filament guide having at least a filament-contacting portion comprising a unicrystalline body of material selected from the group consisting of corundum and spinel, said body having a glossy flame-polished surface.

10. A filament guide comprising a unicrystalline rod of material selected from the group consisting of corundum and spinel, said rod having a bight bent therein for the passage of a filament, said rod having a glossy scratch-free surface substantially identical with the surface produced by intensely heating such a rod.

11. A filament guide comprising a unicrystalline rod composed of a material selected from the group consisting of corundum and spinel, said rod having a glossy, scratch-free, wavy filament contacting surface, said surface being substantially identical with the surface produced by intensely heating such a rod.

MALCOLM H. BARNES.  
EDWARD L. McCANDLESS.

#### REFERENCES CITED

The following references are of record in the file of this patent:

#### UNITED STATES PATENTS

| Number     | Name      | Date           |
|------------|-----------|----------------|
| Re. 12,769 | Palmer    | Mar. 24, 1908  |
| 110,535    | Altemus   | Dec. 27, 1870  |
| 181,394    | Bancroft  | Aug. 22, 1876  |
| 423,847    | White     | Mar. 18, 1890  |
| 1,967,798  | Witte     | July 24, 1934  |
| 2,060,964  | Wider     | Nov. 17, 1936  |
| 2,214,703  | Thurnauer | Sept. 10, 1940 |